

Jan. 7, 1936.

F. L. ANTISELL

2,026,605

METHOD FOR WORKING AND TREATING METALS

Filed Jan. 9, 1933

2 Sheets-Sheet 2

*Fig. 2.*



*Fig. 3.*



*Fig. 6.*



*Fig. 4.*



*Fig. 7.*



INVENTOR

Frank L. Antisell  
by his attorneys  
Byrnes, Stebbins, Parmelee & Blenko

Jan. 7, 1936.

F. L. ANTISELL

2,026,605

METHOD FOR WORKING AND TREATING METALS

Filed Jan. 9, 1933

2 Sheets-Sheet 1

Fig. 1.



Fig. 5.



Fig. 5 A.



Fig. 1A.



Fig. 1B.



INVENTOR

Frank L. Antisell  
by his attorneys  
Byrnes, Stebbins, Parmelee & Blanks

## UNITED STATES PATENT OFFICE

2,026,605

METHOD FOR WORKING AND TREATING  
METALSFrank L. Antisell, Wilkinsburg, Pa., assignor to  
Copperweld Steel Company, Glassport, Pa., a  
corporation of Pennsylvania

Application January 9, 1933, Serial No. 650,913

9 Claims. (Cl. 148—11.5)

My invention relates to a method for working and treating copper or other similar metals and, in particular, copper or other metal which has been deposited electrolytically upon a base of 5 copper or another metal such as steel, and to the formation of a firm bond between the deposited copper and the base metal, as well as between successive deposited layers.

It is well known that copper of an exceedingly 10 high degree of purity, for example, 99.99 percent, can be obtained by electrode position from commercial anodes which, themselves, approach a purity of 99.95 percent. The characteristics of electrolytic copper, however, are not those which 15 are most desirable in the commercial field. Electrolytic copper is characterized by a fairly coarse grain structure, the size of the grains increasing with the thickness of the deposited layer. The initially deposited layers are of very fine structure but subsequently deposited layers show a marked increase in the grain size. The typical grain structure of electrolytic copper is shown in photomicrograph *b* of a plate opposite page 152 of "The Story of Copper" by Watson Davis, published in 1924 by the Century Company, New 20 York, N. Y.

It has not been possible heretofore to improve the grain structure or physical characteristics of electrolytic copper by hot or cold working. It 25 has been found, for example, that the coarse structure characteristic of electrolytic copper has remained even after heating in hydrogen and alternate hot and cold rolling. The bond heretofore obtained between deposited copper and the base metal, furthermore, has not been entirely satisfactory.

I have invented a method for working and treating electrolytic copper which results in a grain structure entirely different from that of 30 the original electrolytic deposit and which gives rise to numerous desirable physical characteristics, principally, high conductivity, with malleability and ductility. I deposit successive layers of copper on the base metal, and mechanically 35 work the layers as deposited to introduce an amorphous constituent into each layer, and by subsequent heat treatment at comparatively low temperatures, very much below the fusion point, I cause an intrusion of the amorphous material 40 into the copper deposit and the base metal forming a tight bond or weld with the latter and equiaxed copper grain structure in the former.

In accordance with my invention, I subject the 45 electrolytic copper to successive cold working operations as the electrolytic deposit proceeds

layer by layer and subsequently heat treat the entire mass of deposited copper at a temperature below the fusion point to bring about finally the desired grain structure and permanent bond to the base. The effect of the mechanical working 5 during the growth of the deposit seems to be a compacting of the copper crystals accompanied by a disintegration of the grains, producing a species of electrolytic copper which is subject to improvement as to grain characteristics by heat 10 treatment. Specifically, I provide for depositing electrolytic copper upon a base in the form of a rod or wire which may be steel or copper. I prefer to rotate the base and move it simultaneously through an electrolytic bath. Upon emergence 15 from the bath, I subject the rotating base with a coating of copper thereon, to the action of rolls disposed axially of the base, provided with a slightly blunted or rounded edge. These edged rolls produce a spiral track on the coated base, 20 the copper in the neighborhood of which is subjected to mechanical working under high pressures. This sequence of electrode position and mechanical working is repeated until the desired 25 thickness of copper has been deposited on the base. The coated base is then ready for heat treatment. I preferably accomplish this by heating the coated base to a final temperature of 1725° F. in a continuous furnace. After heating, the coated base may be rolled at various 30 temperatures as high as 1000° F., depending on the final temper desired, or it may also be drawn through dies.

The increased adherence of the deposit to the base which results from the foregoing process is 35 caused, in my opinion, by an intrusive action of the amorphous grain boundary material of the copper into the intergranular spaces of the base metal. In the welding of wrought iron, mild 40 steel, or other metals, an actual fusion of the metals must occur, accompanied by the formation of a bonding alloy, or the equivalent thereof. The results flowing from my invention may probably be explained on the same basis as the phenomenon of annealing which brings about, at a 45 temperature well below fusion, a grain growth with a corresponding migration or rearrangement of grain boundary material. Such changes favor the intrusive action of foreign grain boundary material, and it is found that there is actually 50 an interchange of such material between the copper and the base at temperatures only slightly above the annealing temperature, resulting in an excellent union of the two metals.

In accordance with my invention, therefore, it 55

is possible to weld two pieces of the same metal or of different metals, by holding them in contact and subjecting them to a temperature much below the fusion point.

- 5 For a complete understanding of the invention and the theory I have evolved to account for the results produced thereby, reference is made to the accompanying drawings illustrating diagrammatically a preferred form of the apparatus 10 for carrying out the method, and the grain structure produced in the electrolytic copper by the invention, as observed in photomicrographs. In the drawings:

15 Figure 1 is a diagrammatic illustration of the electrolytic coating baths, the working rolls and the continuous furnace by which the electrolytic copper is deposited on a base, wire or rod, subjected to mechanical rolling and finally heat treatment, in position thereon;

- 20 Figure 1A is a sectional view along the line IA-IA of Figure 1;

Figure 1B shows generally the appearance of the rod after the first deposit and mechanical working;

- 25 Figure 2 is a partial cross section to greatly enlarged scale taken axially through a copper-clad rod showing the physical effect of the cold working;

30 Figure 3 is a conventional representation of a photomicrograph illustrating the effect of the cold working on the grain structure of the deposited layers;

- 35 Figure 4 is a similar section showing the effect of heat treatment of the coated rod produced according to the invention, showing the effect of heat treatment following the mechanical workings;

40 Figures 5 and 5A are transverse sections showing the effect of the invention on a layer of electrolytic copper deposited on a cast copper base;

Figure 6 shows diagrammatically the crystalline state of the iron and the copper deposited thereon after the mechanical working; and

- 45 Figure 7 is similar to Figure 6 but shows the change in granular structure brought about by heating to temperatures below fusion.

Referring in detail to the drawings, I subject a base member 10, which may be a rod or wire of steel or copper, to treatment in electrolytic 50 baths 11 and 12, each electrolytically deposited layer being subjected to mechanical working in roll stands 13 and 14. After emerging from the last stand of rolls, the coated base passes into a continuous furnace 15 for heat treatment.

- 55 Preferably I provide means for rotating the base during the progress of the coating and heat treating operations. The coated base may easily be wound upon a reel after treatment and the uncoated base unwound from another reel prior to introduction into the baths. Both the unwinding and winding-up reels may be rotated by suitably mounting them, and axial rotation of the rod is thereby effected.

60 The construction of the electrolytic baths 11 and 12, and the method of subjecting the base member to treatment therein, are well known and require no detailed description. The roll stands 13 and 14 each comprise a pair of rolls 16 mounted in suitable housings, not shown. The rolls 16 are shaped so as to have a somewhat rounded or blunted edge 17 and the rolls of each stand are positioned in the housings so as to be slightly offset as illustrated. The shape of the rolls 16 is similar to that resulting from placing 70 a pair of truncated cones base to base. The rolls

16 of each stand are preferably positioned in substantially the same horizontal plane, and are adjusted therein so that the portions of the rolls of greatest diameter are separated by a distance slightly less than the diameter of the coated base. 5 The weight of the coated base thus wedges it between the rolls and, because of the angular relation of the forces involved, the total pressure exerted on the coated member by the rolls is considerable.

10 Because of the shape of the rolls 16, the unit pressure to which the electrolytic copper is subjected is very high. It will be apparent that substantially the total pressure of the rolls on the coated member is transmitted through two 15 spaced points, as shown in Figure 1A.

15 Since the rolls 16 of a single stand are slightly offset in the direction of travel of the base, the result of the cold working in any stand of rolls is to produce helical tracks 18 in the electrolytic 20 layer deposited on the base, as shown in Figure 1B. Succeeding electrolytic treatments, however, cover the helical paths and all other portions of the initially deposited layer and after the second layer is deposited, the mechanical 25 work following thereupon again produces helical tracks.

20 In a particular instance, the dimension of the rolled mark on the wire was .009 inches wide, and the chord of contact is .011 inches, equalling an 30 area of .000099 square inch, or say in round figures .0001 square inch, or a bearing area of one ten thousandths of a square inch.

25 The total weight of wire on point contact is 2.2 pounds, and the resolution of force on this wire 35 by reason of the wedge effect is 5 to 1, resulting in a component of pressure of 5½ pounds, resulting finally in an enormous pressure of 55,000 pounds per square inch on each of the two rollers, thereby compacting the copper completely.

30 Figure 2 illustrates a half section of a length of the base member 10 having five electrolytic layers deposited thereon. The first layer, 19, has a well defined helical track 18 therein formed by the cold rolling after the first electrolytic deposit. 40 The second layer 20 also has a helical track 18 but it is displaced axially of the base 10 relative to the track in the layer 19. It will be observed that the track 18 formed in the initial layer 19 is repeated to a decreasing extent in the succeeding 50 layers. Repeated rolling and electrolytic deposition finally produce a coated base, the surface of which is lightly corrugated, showing a number of helical tracks one overlying the other.

35 Referring in particular to Figure 3, I shall discuss the effect of the cold working on the grain structure of the deposited layers. As shown by the publication referred to above, electrolytic copper is ordinarily of comparatively coarse, columnar grain structure although the layer next 60 the base on which the deposition occurs is usually of finer grain structure than subsequently deposited layers. In Figure 3, I have shown diagrammatically at 19' the grain structure of different portions of the initially deposited layer. 65 This layer, as stated, is of fairly small grain structure but the effect of the cold working to which the layer is subjected by the rolls 16 is to compact the electrolytically deposited copper in the vicinity of the helical track 18 and to refine 70 the grain structure thereof to a marked degree, as indicated by the portion of the layer 19' in alignment with the helical track 18 in the layer 19. It will be understood that the layers 19 and 19' are the same and that at 18 is indicated the 75

actual physical deformation of the deposited layer while at 19' is shown the effect on the grain structure. The portions of the initial layer apart from the track 18 formed therein by the rolls 16 are of comparatively coarse grain structure, as indicated in Figure 3. The coarseness of the layers subsequently deposited increases gradually as previously pointed out.

As described, the helical tracks traced by successive roll stands, such as 13 and 14, are displaced slightly, axially of the base member, and result in the formation of portions of successive layers having similar grain structure disposed in step-like relation as shown in Figure 3. It will thus be apparent that each electrolytic layer is characterized by a helical band of compacted and refined grain structure adjacent the helical track formed by the rolls 16. The remaining band of each layer is of gradually varying grain structure.

After a number of electrolytic depositions and cold rollings, which depends upon the thickness of the coating desired on the finished article, the latter is subjected to heat treatment in the continuous furnace 15 where it is finally heated to approximately 1725° F. This heat treatment brings about a remarkable change in the grain structure of the deposited copper. Instead of separate bands in each layer having different grain characteristics, it is observed that the grain structure of the entire deposited layer is quite fine and uniform. This result I attribute to the intrusive effect of the bands of the deposited layers which have been subjected to cold working. The effect of the axially displaced bands of compacted, fine grain copper in each successive deposited layer seems to spread through adjacent layers by this intrusive action and thereby produce the uniform, fine grain structure which is observed after heat treatment. This is best illustrated in Figure 4 in which it will be observed that the fine grain structure resulting from the cold working of the initial layer in the rolls 16 has spread from the initial layer through adjacent layers to the outside layer. The uniform grain structure shown in Figure 4, of course, is highly desirable since it gives rise to the physical characteristics required in commerce, namely, ductility and malleability, and provides an excellent bond between layers.

Upon emerging from the furnace 15, the coated base may be subjected to smoothing action without substantial reduction in area while hot, by means of either rolls, rotary dies, or other device that does not subject the coat to a great shearing stress, and may thereupon be subjected to any further manufacturing operations desirable. Since, as explained above, the union is effected by the migration of amorphous material, great welding pressures are not necessary or desirable. By bringing the two metals in contact at high temperature without friction, it is possible to work the composite article by tandem devices spaced apart so that when wire reaches the second device it can be reduced by about 20%, thereby carrying out the two operations of uniting and reducing at no extra cost.

I have also observed that the intrusive action above mentioned is also effective in the case of, for example, a steel billet having a copper sheath cast thereon, and a second copper sheath deposited electrolytically on the first. Cast copper, as well as electrolytic copper, has a very definite and well recognized type of grain structure. By sub-

jecting the electrolytic layer deposited on a cast copper sheath to combined mechanical working and heat treatment, as above described, however, I am able to convert the grain structure of the electrolytic copper and also that of the cast copper sheath to substantially the type shown in Figure 4, resulting in a single homogeneous grain structure throughout the copper layers, demonstrating the remarkable effects of the intrusive action of the amorphous constituent. Figures 5 10 and 5A show diagrammatically the grain structure of electrolytic and cast copper before and after subjecting them to the process of my invention.

The effect of the treatment described upon the grain structure of the copper-iron boundary is best shown in Figures 6 and 7. In Figure 6, the iron has a fairly coarse grain structure and the copper has the grain structure illustrated more particularly in Figure 3. The solid circles in Figure 6 represent the amorphous constituent as shown in Figure 3 at 19'. In Figure 7, the iron base is unaltered as to grain orientation. The copper grain structure has become equiaxed. The amorphous constituent has disappeared with an inter-copper penetration at all grain boundaries of the iron and with interface penetration or, more strictly speaking, inter-crystalline penetration of the Neumann bands that appears to be, in effect, interface penetration. On heating the composite article to a temperature between 400° and 800° F., however, the grain structure is converted into that shown in Figure 7. It will be apparent that the grain boundary material of the copper has penetrated into the intergranular spaces of the iron and that, simultaneously, the grain structure of the copper has been considerably refined. There is an annealing effect upon the iron grain structure characterized by the introduction of Neumann lines. The interlocking grain boundary material, of course, effects a very strongly adherent union between the copper and the iron. The net effect of the electrodeposition followed by mechanical working and heat treatment at about 800° F., seems to be that a weld between the metals is produced at a temperature much below the fusion point. There appears to be a critical temperature, at about the annealing point, at which this result occurs.

It will be apparent from the foregoing description that the invention provides a highly useful method and apparatus for making electrolytic copper subject to heat treatment for improving the physical characteristics thereof, including the bond with the base, whereas heretofore it has been impossible to bring about any improvement in electrolytic copper by heat treatment. My invention makes it possible to obtain a marked improvement in the characteristics not only of electrolytic copper, but also of other metals of similar properties, by a simple heat treatment and hot working preceded by the mechanical working after the deposition of each layer, as described above.

The dimension of the unit of amorphous material is of the order of a small multiple of atomic diameters. The ordinary grain boundary is from one to one-hundred thousand times that size and provides, therefore, a space for many millions of the amorphous units when the metal is below the temperature at which grain growth prevails. On subjecting the metal to temperatures approaching the time-temperature annealing value, the tendency to form solid solutions within the matrix, as well as the inherent tendency for the amorphous

material to recrystallize into grain units, will bring the intrusive action to an end when the grain size becomes larger than the grain boundaries of the adjacent metal. While the size of the amorphous units must approximate only a fraction of the dimensions of the grain boundary, the so-called interface penetration which may be, in fact, intrusions in the Neumann bands, must be of the order of atomic diameters. If interface penetration is effected, it must follow that not only must the grain boundary material be amorphous but it must be so manipulated regarding time and temperature as to extend the time of intrusive action to the point where the adjacent metals are saturated.

The amorphous constituent may be provided in ways other than that already described. As an example, I may wash the coated rod with nickel, arsenic or other solutions as it emerges from the electrolytic baths, thus introducing a foreign constituent of .001%.

Although I have illustrated and described herein but one preferred embodiment of the invention, it will be obvious that many changes may be made in the apparatus and method disclosed herein without departing from the scope of the invention or the spirit of the appended claims.

I claim:

1. The method of making a copper sheathed wire including the steps of depositing successive layers of copper from an electrolytic solution of copper onto a core wire, intermediate the depositing of successive layers compacting spaced paths on the layer already deposited leaving uncompacted portions therebetween, and annealing the composite article without reaching the fusion point of the copper layers.

2. A method of making a coherent, integral mass of metal from a series of layers thereof including the steps of successively compacting portions of each layer to refine the grain structure thereof, leaving the intermediate portions in their original coarse-grained state to anchor the layers together, and annealing the layers whereby the intrusive effect of the compacted portions extends to adjacent layers wiping out boundaries therebetween and uniting the layers.

3. The method of making a composite article, which comprises electrodepositing successive layers of metal on a core, compacting spaced portions of each layer and leaving uncompacted portions therebetween before depositing the succeeding layer, and annealing the article to refine the grain structure and cause the intrusive effect of the compacted portions to extend to adjacent layers.

4. The method of making a composite article, which comprises electrodepositing successive layers of metal on a core, rotating the article

axially while advancing it longitudinally in contact with compacting rollers to compact spaced portions of each layer and leaving uncompacted portions therebetween before depositing the succeeding layer, and annealing the article to refine the grain structure and cause the intrusive effect of the compacted portions to extend to adjacent layers.

5. The method of making a composite article, which comprises electrodepositing successive layers of copper on a steel core, compacting spaced portions of each deposited layer and leaving uncompacted portions therebetween before depositing the succeeding layer, and annealing the article to refine the grain structure and cause the intrusive effect of the compacted portions to extend to adjacent layers.

6. The method of making a composite article which comprises electrolytically depositing a copper layer from a copper solution onto a base metal, compacting spaced paths thereon while leaving uncompacted portions therebetween, thereafter electrodepositing another layer of copper, and annealing the composite article without reaching the fusion point of the copper layers.

7. The method of making a composite article which comprises passing an elongate core such as a wire as a cathode through an electrolytic bath so as to deposit a copper layer on the core, forming compacted spaced paths in the form of helices on the deposited copper while leaving uncompacted portions therebetween, thereafter effecting the electrodeposition of further copper on the preceding layer, and annealing the composite article without reaching the fusion point of the copper layers.

8. The method of making a copper sheathed wire which comprises passing a core wire as a cathode through an electrolytic bath, rotating the wire axially while advancing it through the bath, forming compacted helical paths on the deposited metal while leaving uncompacted portions therebetween, thereafter continuing the electrodeposition of an additional layer of copper, and annealing the composite article without reaching the fusion point of the copper layers.

9. The method of producing a copper sheathed wire including the steps of electrodepositing successive layers of copper on a core wire, axially rotating the coated wire and while rotating it forming helical depressions or slight grooves in the deposited metal and leaving uncompacted portions therebetween before depositing the succeeding layer, and annealing the copper sheathed wire without reaching the fusion point of the copper layers.

FRANK L. ANTISELL.